# EUROPEAN PATENT SPECIFICATION

(11) **EP 3 034 211 B1**
(45) Date of publication and mention of the grant of the patent: **29.07.2026**
(21) Application number: 14198569.7
(22) Date of filing: 17.12.2014
(51) Int. Cl.: B22F 3/15, C22C 33/02, C22C 38/22, C21D 6/02, C22C 38/00, C22C 38/02, C22C 38/04, C22C 38/12, C22C 38/24, C22C 38/32

(54) **A WEAR RESISTANT TOOL STEEL PRODUCED BY HIP**
VERSCHLEIßFESTER, DURCH HEIßISOSTATISCHES PRESSEN GEFERTIGTER, WERKZEUGSTAHL
ACIER À OUTIL RÉSISTANT À L'USURE PRODUIT PAR PRESSAGE ISOSTATIQUE À CHAUD

(43) Date of publication of application: 22.06.2016
(73) Proprietor: Uddeholms AB, 683 85 Hagfors (SE)
(72) Inventor: Tidesten, Magnus, 683 34 Hagfors (SE)
(74) Representative: Noréns Patentbyrå AB

(56) References cited:
- GB-A- 2 187 757
- JP-A- 2002 022 891
- JP-A- H07 179 997
- US-A- 4 318 733

## Description

### TECHNICAL FIELD

The invention relates to a wear resistant tool steel produced by HIP. The tool steel is alloyed with boron.

### BACKGROUND OF THE INVENTION

Nitrogen and vanadium alloyed powder metallurgy (PM) tool steels attained a considerable interest because of their unique combination of high hardness, high wear resistance and excellent galling resistance. These steels have a wide rang of applications where the predominant failure mechanisms are adhesive wear or galling. Typical areas of application include blanking and forming, fine blanking, cold extrusion, deep drawing and powder pressing. The basic steel composition is atomized, subjected to nitrogenation and thereafter the powder is filled into a capsule and subjected to hot isostatic pressing (HIP) in order to produce an isotropic steel. A high performance steel produced in this way is described in WO 00/79015 A1.

Although the known steel has a very attractive property profile there is a continuous strive for improvements of the tool material in order to further improve the surface quality of the products produced as well as to extend the tool life, in particular under severe working conditions, where galling is the main problem.

JPH07179997 discloses a high speed steel type powder alloy. This high speed steel type powder alloy has a chemical composition consisting of, by weight, 0.3-3.5% C, 0.6-3.5% Si, <=0.6% Mn, 0.5-2.9% Cr, 7.0-50% Mo, 0.5-20.0% W, 0.5-12.0%, in total, of one or more elements among V, Ti, Nb, and Ta, 0.1-5.0% B, and the balance essentially Fe. Further, besides these alloy components, 7.0-20% Co and/or <=3.0% Ni can be incorporated.

### DISCLOSURE OF THE INVENTION

The object of the present invention is to provide powder metallurgy (PM) produced tool steel having an improved property profile for advanced cold working like fine blanking.

Another object of the present invention is to provide a powder metallurgy (PM) produced tool steel having a composition and microstructure leading to improvements in the surface quality of the produced parts.

The foregoing objects, as well as additional advantages are achieved to a significant measure by providing a tool steel having a composition as set out in the claims.

The invention is defined in the claims.

### DETAILED DESCRIPTION

The present invention relates to a HIPed tool steel comprising a hard phase consisting mainly of multiple borides containing Fe in a hardenable matrix. The double boride is of the type M₂M'B₂, where M and M' stand for metals of the multiple boride. Said boride forming elements are generally selected from Cr, Mo, W, Ti, V, Nb, Ta, Hf and Co. In the present case M is Mo and M' is Fe. However, the boride may contain substantial amounts of one ore more of the other boride forming elements. However, in the following the double boride will simply be referred to as Mo₂FeB₂ although the boride also may contain Ni and one or more of the above mentioned boride forming elements.

The importance of the separate elements and their interaction with each other as well as the limitations of the chemical ingredients of the claimed alloy are briefly explained in the following. All percentages for the chemical composition of the steel are given in weight % (wt. %) throughout the description. The upper and lower limits of the individual elements may be freely combined within the limits set out in claim 1.

### Carbon (0.2 - 1.5 %)

Carbon is to be present in a minimum content of 0.2 %, preferably 0.3 % or 0.35 %. The upper limit for carbon is 1.5 %. Carbon is important for the formation of carbides and for the hardening Preferably, the carbon content is adjusted in order to obtain 0.4-0.6 % C dissolved in the matrix at the austenitizing temperature. In any case, the amount of carbon should be controlled such that the amount of carbides of the type M₂₃C₆, M₇C₃, M₆C and MC in the steel is limited. The upper limit may therefore be set to 0.8, 0.6, 0.5 or 0.45 %

### Chromium (2.8 - 25 %)

Chromium is an optional component. However, Cr is for most applications present in contents of at least 2.8 % in order to provide a sufficient hardenability. Cr is preferably higher for providing a good hardenability in large cross sections during heat treatment. If the chromium content is too high, this may lead to the formation of undesired carbides, such as M₇C₃. In addition, this may also increase the propensity of retained austenite in the microstructure. The lower limit may be 3.4 % or 4.2 The upper limit may be 6.0, 5.4 %, or 4,6 %. On the other hand, Chromium contents of mare then 10 %, preferably more than 12 % are used for stainless applications.

### Molybdenum (12 - 35 %)

Mo is the main element forming the hard boride. In the present invention, a high amount of Molybdenum is used in order to obtain a desired precipitation of the boride Mo₂FeB₂ in an amount of 5-35 vol. %. Preferred ranges include 12-30 % and 15-25%. Mo is also known to have a very favourable effect on the hardenability is essential for attaining a good secondary hardening response. For this reason it is preferred that the amount of Mo remaining in the matrix after quenching form 1100°C is 1.5-2.5 %.

### Boron (0.7 - 3 %)

Boron, which is the main hard phase-forming element, should be at least 0.7 % so as to provide the minimum amount of 5 % hard phase Mo₂FeB₂. The amount of B is limited to 3 % for not making the alloy to brittle.

### Tungsten (≤ 3 %)

The effect of tungsten is similar to that of Mo. However, for attaining the same effect it is necessary to add twice as much W as Mo on a weight % basis. Tungsten is expensive and it also complicates the handling of scrap metal. The maximum amount is therefore limited to 3 %, preferably 1%, more preferably 0.3 % and most preferably W is not deliberately added at all.

### Vanadium (≤ 15 %)

Vanadium forms evenly distributed primary and secondary precipitated carbides of the type MC. In the inventive steel M is mainly vanadium but Cr and Mo may be present to some extent. The maximum addition of V is restricted to 15 % and the preferred maximum amount is 5 %. However, in the present case V is mainly added for obtaining a desired composition of the steel matrix before hardening. The addition may therefore be limited to 2.0 % or even to 0.5 %. A preferred range is 0.1-0.5 % V.

### Niobium (≤ 15 %)

Niobium is similar to vanadium in that it forms MC. However, for attaining the same effect it is necessary to add twice as much Nb as V on a weight % basis. Nb also results in a more angular shape of the MC. Hence, the maximum addition of Nb is restricted to 15 % and the preferred maximum amount is 5 %. Preferably, no niobium is added.

### Silicon (0.1 - 2.5 %)

Silicon is used for deoxidation. Si also increases the carbon activity and is beneficial for the machinability. Si is therefore present in an amount of 0.1 - 2.5 %. For a good deoxidation, it is preferred to adjust the Si content to at least 0.2 %. The lower limit may be set to 0.3 %, 0.35 % or 0.4 %. However, Si is a strong ferrite former and should be limited to 2.5 %. The upper limit may be set to 1.5%, 1 %, 0.8 %, 0.7 % or 0.6 %. A preferred range is 0.2 - 0.8 %.

### Manganese (0.1 - 2.5 %)

Manganese contributes to improving the hardenability of the steel and together with sulphur manganese contributes to improving the machinability by forming manganese sulphides. Manganese shall therefore be present in a minimum content of 0.1 %, preferably at least 0.2 %. At higher sulphur contents manganese prevents red brittleness in the steel. The steel shall contain maximum 2.5 % Mn. The upper limit may be set to 1.5 %, 1.2 %, 1.0 %, 0.8 % or 0.6%. However, preferred ranges are 0.2 - 0.8 % and 0.2 - 0.6 %.

### Nickel (≤ 5%)

Nickel is optional and may be present in an amount of not more than 5 %. It gives the steel a good hardenability and toughness. Because of the expense, the nickel content of the steel should be limited as far as possible. Accordingly, the Ni content is preferably limited to 2%, more preferably to 1.0% or 0.3%.

### Copper (≤ 3.0%)

Cu is an optional element, which may contribute to increasing the hardness and the corrosion resistance of the steel. If used, the preferred range is 0.02 - 2% and the most preferred range is 0.04 - 1.6%. However, it is not possible to extract copper from the steel once it has been added. This drastically makes the scrap handling more difficult. For this reason, Copper is normally not deliberately added.

### Cobalt (≤ 10 %)

Co is an optional element, which may be present in an amount of not more than 10 %. Co dissolves in iron (ferrite and austenite) and strengthens it whilst at the same time imparting high temperature strength. Co increases the Mₛ temperature. Co can substitute mainly Fe in the Mo₂FeB₂ boride. A preferred maximum content is 2 %. However, scrap handling will be more difficult. For this reason, Co is not deliberately added

### Ti, Ta, Zr and Hf

These elements are boride and carbide formers and may be present in the alloy in the claimed ranges for altering the composition of the hard phases. However, normally none of these elements are added.

### Phosphorous

P is an impurity element and a solid solution strengthening element. However, P tends to segregate to the grain boundaries, reduces the cohesion and thereby the toughness. P is therefore normally limited to ≤ 0.05 %.

### Sulphur (≤ 0.5%)

S contributes to improving the machinability of the steel. At higher sulphur contents there is a risk for red brittleness. Moreover, a high sulphur content may have a negative effect on the fatigue properties of the steel. The steel shall therefore contain ≤ 0.5 %, preferably ≤ 0.03 %.

### EXAMPLE (Not forming part of the invention)

10 kg of an alloy having the composition given below was melted in a laboratory furnace and subjected to Ar-gas atomizing.

| | |
|---|---|
| C | 0.3 |
| Si | 0.3 |
| Mn | 0.3 |
| Mo | 19 |
| B | 2.1 |
| Fe | balance. |

The powder was sieved to < 500 µm, filled in steel capsules having a diameter of 63 mm and a height of 150 mm. HIPing was performed at a temperature of 1150 °C, the holding time was 2 hours and the pressure 110 MPa. The cooling rate was < 1 °C/s. The material thus obtained was forged at 1130 °C to the dimension 20x30 mm. Soft annealing was performed at 900 °C with a cooling rate of 10 °C/h down to 750 °C and thereafter cooling freely in air. Hardening was performed by austenitizing at 1100 °C for 30 minutes followed by quenching in water followed by tempering. The result of the hardness testing after tempering is given in Table 1.

The amount of the hard phase was found to be 24 vol. % and the borides were found to have a small size. The area fraction of borides in different size classes is given in Table 2 below.

**Table. 1. Hardness as a function of the tempering temperature after hardening from 1100 °C.**

| Tempering temperature (°C) | Hardness HRC |
|---|---|
| 200 | 60 |
| 300 | 56 |
| 400 | 54 |
| 500 | 53 |
| 525 | 53 |
| 550 | 54 |
| 600 | 49 |

**Table. 2. Size distribution of the borides.**

| Size range (µm) | Area fraction (%) |
|---|---|
| 0-1 | 6.3 |
| 1-2 | 13.5 |
| 2-3 | 4.0 |
| 3-4 | 0.2 |

The microstructure is shown in Fig. 1. The high area fraction and the uniform distribution of the Mo₂FeB₂ borides results in a material having excellent anti-galling properties such that it would be possible to dispense with surface treatments like PVD, CVD and TD.

### INDUSTRIAL APPLICABILITY

The tool steel of the present invention is particular useful in applications requiring very high galling resistance.

## Claims

1. A tool steel produced by powder metallurgy and hot isostatic pressing resulting in that the steel is isotropic has a non-amorphous microstructure and has a density of > 98 % of the theoretical density (TD), the steel consists of in weight % (wt.%):
| | |
|---|---|
| C | 0.2 - 1.5 |
| Si | 0.1 - 2.5 |
| Mn | 0.1 - 2.5 |
| Mo | 12-35 |
| B | 0.7 - 3 |
| Cr | 2.8 - 25 |
| V | ≤ 15 |
| Nb | ≤ 15 |
| Ti | ≤ 1 |
| Ta | ≤ 5 |
| Zr | ≤ 5 |
| Hf | ≤ 5 |
| Ni | ≤ 5 |
| Co | ≤ 10 |
| Cu | ≤ 3 |
| W | ≤ 3 |
| S | ≤ 0.5 |
Fe and impurities balance,
wherein the steel comprises 5 - 35 volume % hard phase, wherein the hard phase comprises at least one of borides, nitrides, carbides and/or combinations thereof and wherein the maximal Equivalent Circle Diameter of the hard phase is less than 5 µm.

2. A steel according to claim 1, wherein the steel fulfils at least one of the following conditions,
| | |
|---|---|
| C | 0.3 - 0.6 |
| Si | 0.2 - 1.5 |
| Mn | 0.2 - 1.5 |
| Mo | 12 - 30 |
| B | 0.7 - 2.5 |

3. A steel according to claim 1 or 2, wherein the steel fulfils at least one of the following conditions
| | |
|---|---|
| Cr | ≤ 20 |
| V | ≤ 5 |
| Nb | ≤ 5 |
| Ta | ≤ 1 |
| Zr | ≤ 1 |
| Hf | ≤ 1 |
| Ni | ≤ 2 |
| Co | ≤ 2 |
| Cu | ≤ 1 |
| W | ≤ 1 |
| S | ≤ 0.03 |

4. A steel according to any of the preceding claims, wherein the steel fulfils at least one of the following conditions
| | |
|---|---|
| C | 0.3 - 0.5 |
| Si | 0.2 - 0.8 |
| Mn | 0.2 - 0.8 |
| Mo | 15 - 25 |
| B | 1.8 - 2.2 |
| Cr | 3.0 - 16 |
| V | 0.1 - 2.0 |

5. A steel according to any of the preceding claims, wherein the steel fulfils at least one of the following conditions
| | |
|---|---|
| C | 0.35 - 0.45 |
| Si | 0.2 - 0.6 |
| Mn | 0.2 - 0.6 |
| Cr | 3.0 - 6.0 |
| V | 0.1 - 0.5 |

6. A steel according to any of claims 1-4, wherein the steel fulfils at least one of the following conditions
| | |
|---|---|
| C | 0.35 - 0.45 |
| Si | 0.2 - 0.6 |
| Mn | 0.2 - 0.6 |
| Cr | 10.0 - 15.0 |
| V | 0.1 - 0.5 |

7. A steel according to any of the preceding claims, wherein the steel fulfils at least one of the following conditions
| | |
|---|---|
| V | 0.2 - 0.4 |
| P | < 0.05 |
| S | < 0.003 |
| O | < 0.005 |

8. A steel according to any of claims 1-4, wherein the metallic matrix fulfils the following requirements after quenching from 1100 °C
| | |
|---|---|
| C | 0.4 - 0.5 |
| Si | 0.3 - 0.5 |
| Mn | 0.3 - 0.5 |
| Mo | 1.5 - 2.5 |
| Cr | 4.0 - 5-0 |
| V | 0.3 - 0.4 |

9. A steel according to any of the preceding claims, wherein the maximal Equivalent Circle Diameter of the hard phase is less than 3 µm.

10. A steel according to any of the preceding claims, wherein the steel comprises 15 - 25 volume % hard phase and wherein the maximal Equivalent Circle Diameter of the hard phase is less than 3 µm.

## Patentansprüche

1. Werkzeugstahl, hergestellt durch Pulvermetallurgie und heißisostatisches Pressen, wobei es sich ergibt, dass der Stahl isotrop ist, eine nicht amorphe Mikrostruktur aufweist und eine Dichte von > 98 % der theoretischen Dichte (TD) aufweist, wobei der Stahl in Gewichtsprozent (Gew.-%) besteht aus:
| | |
|---|---|
| C | 0,2 - 1,5 |
| Si | 0,1 - 2,5 |
| Mn | 0,1 - 2,5 |
| Mo | 12 - 35 |
| B | 0,7 - 3 |
| Cr | 2,8 - 25 |
| V | ≤ 15 |
| Nb | ≤ 15 |
| Ti | ≤ 1 |
| Ta | ≤ 5 |
| Zr | ≤ 5 |
| Hf | ≤ 5 |
| Ni | ≤ 5 |
| Co | ≤ 10 |
| Cu | ≤ 3 |
| W | ≤ 3 |
| S | ≤ 0,5 |
Rest Fe und unvermeidbare Verunreinigungen,
wobei der Stahl 5 - 35 Vol.-% Hartphase umfasst, wobei die Hartphase mindestens eines aus Boriden, Nitriden, Karbiden und / oder Kombinationen davon umfasst und wobei der maximale äquivalente Kreisdurchmesser der Hartphase weniger als 5 µm beträgt.

2. Stahl nach Anspruch 1, wobei der Stahl mindestens eine der folgenden Bedingungen erfüllt:
| | |
|---|---|
| C | 0,3 - 0,6 |
| Si | 0,2 - 1,5 |
| Mn | 0,2 - 1,5 |
| Mo | 12 - 30 |
| B | 0,7 - 2,5 |

3. Stahl nach Anspruch 1 oder 2, wobei der Stahl mindestens eine der folgenden Bedingungen erfüllt,
| | |
|---|---|
| Cr | ≤ 20 |
| V | ≤ 5 |
| Nb | ≤ 5 |
| Ta | ≤ 1 |
| Zr | ≤ 1 |
| Hf | ≤ 1 |
| Ni | ≤ 2 |
| Co | ≤ 2 |
| Cu | ≤ 1 |
| W | ≤ 1 |
| S | ≤ 0,03 |

4. Stahl nach einem der vorstehenden Ansprüche, wobei der Stahl mindestens eine der folgenden Bedingungen erfüllt,
| | |
|---|---|
| C | 0,3 - 0,5 |
| Si | 0,2 - 0,8 |
| Mn | 0,2 - 0,8 |
| Mo | 15 - 25 |
| B | 1,8 - 2,2 |
| Cr | 3,0 - 16 |
| V | 0,1 - 2,0 |

5. Stahl gemäß einem der vorstehenden Ansprüche, wobei der Stahl mindestens eine der folgenden Bedingungen erfüllt,
| | |
|---|---|
| C | 0,35 - 0,45 |
| Si | 0,2 - 0,6 |
| Mn | 0,2 - 0,6 |
| Cr | 3,0 - 6,0 |
| V | 0,1 - 0,5 |

6. Stahl nach einem der Ansprüche 1-4, wobei der Stahl mindestens eine der folgenden Bedingungen erfüllt,
| | |
|---|---|
| C | 0,35 - 0,45 |
| Si | 0,2 - 0,6 |
| Mn | 0,2 - 0,6 |
| Cr | 10,0 - 15,0 |
| V | 0,1 - 0,5 |

7. Stahl nach einem der vorstehenden Ansprüche, wobei der Stahl mindestens eine der folgenden Bedingungen erfüllt,
| | |
|---|---|
| V | 0,2 - 0,4 |
| P | < 0,05 |
| S | < 0,003 |
| O | < 0,005 |

8. Stahl nach einem der Ansprüche 1-4, wobei die metallische Matrix nach dem Abschrecken aus 1100 °C die folgenden Anforderungen erfüllt,
| | |
|---|---|
| C | 0,4 - 0,5 |
| Si | 0,3 - 0,5 |
| Mn | 0,3 - 0,5 |
| Mo | 1,5 - 2,5 |
| Cr | 4,0 - 5,0 |
| V | 0,3 - 0,4 |

9. Stahl nach einem der vorstehenden Ansprüche, wobei der maximale äquivalente Kreisdurchmesser der Hartphase kleiner als 3 µm ist.

10. Stahl nach einem der vorstehenden Ansprüche, wobei der Stahl 15 - 25 Vol.-% Hartphase umfasst und wobei der maximale äquivalente Kreisdurchmesser der Hartphase weniger als 3 µm beträgt.

## Revendications

1. Un acier pour outils produit par métallurgie des poudres et pressage isostatique à chaud, résultant en le fait que l'acier est isotropique, a une microstructure non-amorphe et a une densité supérieure à 98 % de la densité théorique (TD), l'acier se composant, en pourcentage massique (% en poids) de :
| | |
|---|---|
| C | 0,2 - 1,5 |
| Si | 0,1 - 2,5 |
| Mn | 0,1 - 2,5 |
| Mo | 12 - 35 |
| B | 0,7-3 |
| Cr | 2,8 - 25 |
| V | ≤ 15 |
| Nb | ≤ 15 |
| Ti | ≤ 1 |
| Ta | ≤ 5 |
| Zr | ≤ 5 |
| Hf | ≤ 5 |
| Ni | ≤ 5 |
| Co | ≤ 10 |
| Cu | ≤ 3 |
| W | ≤ 3 |
| S | ≤ 0,5 |
le reste en Fe et en impuretés,
l'acier comprenant de 5 à 35 % en volume de phase dure, la phase dure comprenant au moins un parmi : borures, nitrures, carbures et/ou des combinaisons de ceux-ci, et le diamètre équivalent maximal de la phase dure étant inférieur à 5 µm.

2. Acier selon la revendication 1, l'acier remplissant au moins une des conditions suivantes :
| | |
|---|---|
| C | 0,3 - 0,6 |
| | |
|---|---|
| Si | 0,2 - 1,5 |
| Mn | 0,2 - 1,5 |
| Mo | 12 - 30 |
| B | 0,7 - 2,5 |

3. Acier selon la revendication 1 ou la revendication 2, l'acier remplissant au moins une des conditions suivantes :
| | |
|---|---|
| Cr | ≤ 20 |
| V | ≤ 5 |
| Nb | ≤ 5 |
| Ta | ≤ 1 |
| Zr | ≤ 1 |
| Hf | ≤ 1 |
| Ni | ≤ 2 |
| Co | ≤ 2 |
| Cu | ≤ 1 |
| W | ≤ 1 |
| S | ≤ 0,03 |

4. Acier selon l'une quelconque des revendications précédentes, l'acier remplissant au moins une des conditions suivantes :
| | |
|---|---|
| C | 0,3 - 0,5 |
| Si | 0,2 - 0,8 |
| Mn | 0,2 - 0,8 |
| Mo | 15 - 25 |
| B | 1,8 - 2,2 |
| Cr | 3,0 - 16 |
| V | 0,1 - 2,0 |

5. Acier selon l'une quelconque des revendications précédentes, l'acier remplissant au moins une des conditions suivantes :
| | |
|---|---|
| C | 0,35 - 0,45 |
| Si | 0,2 - 0,6 |
| Mn | 0,2 - 0,6 |
| Cr | 3,0 - 6,0 |
| V | 0,1 - 0,5 |

6. Acier selon l'une quelconque des revendications 1 à 4, l'acier remplissant au moins une des conditions suivantes :
| | |
|---|---|
| C | 0,35 - 0,45 |
| Si | 0,2 - 0,6 |
| Mn | 0,2 - 0,6 |
| Cr | 10,0 - 15,0 |
| V | 0,1 - 0,5 |

7. Acier selon l'une quelconque des revendications précédentes, l'acier remplissant au moins une des conditions suivantes
| | |
|---|---|
| V | 0,2 - 0,4 |
| P | < 0,05 |
| S | < 0,003 |
| O | < 0,005 |

8. Acier selon l'une quelconque des revendications 1 à 4, dans lequel la matrice métallique satisfait aux exigences suivantes après trempe à partir de 1100°C
| | |
|---|---|
| C | 0,4 - 0,5 |
| Si | 0,3 - 0,5 |
| Mn | 0,3 - 0,5 |
| Mo | 1,5 - 2,5 |
| Cr | 4,0 - 5,0 |
| V | 0,3 - 0,4 |

9. Acier selon l'une quelconque des revendications précédentes, dans lequel le diamètre équivalent maximal de la phase dure est inférieur à 3 µm.

10. Acier selon l'une quelconque des revendications précédentes, dans lequel l'acier comprend 15 à 25 % en volume de phase dure et dans lequel le diamètre équivalent maximal de la phase dure est inférieur à 3 µm.
